

# UNITED STATES PATENT OFFICE.

JOSEPH LÉON MARIE ALPHONSE REIS, OF ANTWERP, BELGIUM.

## COMPOSITION FOR PREVENTING BOILER INCRUSTATIONS.

SPECIFICATION forming part of Letters Patent No. 655,119, dated July 31, 1900.

Application filed June 28, 1899. Serial No. 721,607. (No specimens.)

*To all whom it may concern:*

Be it known that I, JOSEPH LÉON MARIE ALPHONSE REIS, a subject of the King of Belgium, residing at Antwerp, in the Kingdom of Belgium, have invented certain new and useful Improvements in Means for Preventing Incrustations in Steam-Boilers, of which the following is a specification.

The means now employed for preventing the formation of deposits and incrustations in steam-boilers can ordinarily only prevent salts of lime, magnesia, or iron from adhering to the walls of the boiler, but are not capable of avoiding deposits of such matters in the boiler in the condition of mud, and to remove such muddy sediments wholly it is always necessary to draw off all the water contained in the boiler and to open the boiler itself. Now this invention is intended to obviate these inconveniences; and it consists in keeping the salts which the water in the boiler contains in a state of solution until a very high degree of concentration is reached, so that complete saturation does not set in until after the boiler has been in operation for a comparatively-protracted space of time. When a sufficient saturation of the water in the boiler has been obtained, which may be ascertained by drawing off a little of the water from the boiler into a test tube or gage and determining the specific gravity of the water (after it has called down) by means of Baumé's salinometer, all that is required is to discharge the water from the boiler without any fear of the boiler retaining any muddy sediments, and consequently without the necessity of opening and inspecting the boiler. In practice it may be held down as a rule, that the water is sufficiently saturated, when it attains 15° Baumé, though saturation may be carried much further and allowed to rise to at least 25° Baumé or a density of 120° and a composition showing about thirty per cent. of sedimentary salts. The time during which operation may be thus conducted without discharging the contents of the boiler may vary, according to the nature of the water employed and the capacity of the boiler, between a fortnight and three months. By the use of my improved composition or preparation it is

possible for the boiler to be maintained in operation for an unlimited period without any waste of time and without the expense for labor which the disconnection and refitting of the joints and the cleansing of the interior of the boiler would otherwise involve. Besides as the boiler at all times remains clean any loss of fuel is obviated and any danger of explosion averted.

In carrying out my invention in practice in order to maintain the salts contained in the boiler-water in a state of solution I make use of a special preparation consisting of, first, sugar, no matter what its origin, or any saccharine substance, such as molasses from sugar factories; second, extract of tannin; third, silicate of soda or of potash; fourth, boric acid, and, fifth, the quantity of water necessary for binding these ingredients together. The proportions of the ingredients may vary according to circumstances. In practice, however, I prefer to employ the ingredients in substantially the following proportions: sugar, fifty-eight parts; extract of tannin, twenty parts; silicate, twenty parts; boric acid, two parts. The quantity of water with which the above ingredients may be mixed will of course vary with the nature of the water used in the boiler. After admitting the compound thus formed in the boiler the water contained therein, whatever its percentage of salts of lime, should remain limpid, though slightly colored, and no precipitate can form, even in the presence of a large quantity of sea-salt.

By the employment of the novel preparation hereinabove described the formation of adhesive incrustations and, indeed, the collection of heavy solidifying muddy deposits, which cannot be got rid of by simply emptying the boiler, but invariably require the boiler to be opened, will in all cases be avoided, whatever the nature of the water used.

What I claim is—

1. The herein - described composition for preventing incrustations in steam-boilers, the same consisting of sugar, extract of tannin, silicate of soda or of potash, boric acid and sufficient water necessary for binding the above ingredients, substantially as described.

2. The herein - described composition for  
preventing incrustations in steam-boilers, the  
same consisting of fifty - eight (58) parts of  
sugar, twenty (20) parts of extract of tannin,  
5 twenty (20) parts of silicate, two (2) parts of  
boracic acid and water sufficient to bind the  
above ingredients.

In witness whereof I have hereunto set my  
hand in presence of two witnesses.

JOSEPH LÉON MARIE ALPHONSE REIS.

Witnesses:

FRANCIS HAMILTON,  
H. CHRISTIAENSEN.